

Nov. 12, 1968

H. S. AVERY ET AL

3,410,682

ABRASION RESISTANT CHROMIUM-MOLYBDENUM CAST IRONS

Filed Sept. 11, 1967

3 Sheets-Sheet 1



Fig. 1

"WSAF" TEST

Inventors

Howard S. Avery  
Henry J. Chapin

By Wallace, Kinzer and Dorn  
Attorneys

Nov. 12, 1968

H. S. AVERY ET AL

3,410,682

ABRASION RESISTANT CHROMIUM-MOLYBDENUM CAST IRONS

Filed Sept. 11, 1967

3 Sheets-Sheet 2



Fig. 4



Fig. 3



Fig. 2

Inventors

Howard S. Avery  
Henry J. Chapin

By Wallace, Kinger and Dorn  
Attorneys

Nov. 12, 1968

H. S. AVERY ET AL

3,410,682

ABRASION RESISTANT CHROMIUM-MOLYBDENUM CAST IRONS

Filed Sept. 11, 1967

3 Sheets-Sheet 3

Fig. 6



Fig. 5



Inventors

Howard S. Avery  
Henry J. Chapin

By Wallace, Kinzer and Domi  
Attorneys

3,410,682

**ABRASION RESISTANT CHROMIUM-MOLYBDENUM CAST IRONS**

Howard S. Avery and Henry J. Chapin, Mahwah, N.J., assignors to Abex Corporation, New York, N.Y., a corporation of Delaware

Continuation-in-part of application Ser. No. 403,314, Oct. 12, 1964. This application Sept. 11, 1967, Ser. No. 667,628

12 Claims. (Cl. 75—128)

**ABSTRACT OF THE DISCLOSURE**

Abrasion resistant cast iron alloys consisting essentially of 2.5 to 3.4% carbon, 0.15 to 1.6% nickel, 12.5—25.6% chromium, 0.38 to 2.90% molybdenum, and the balance iron. A second species contains 2.5 to 3.2% carbon, 0.4 to 2.1% manganese, 0.1 to 1.9% nickel, 15 to 23% chromium, 0.4 to 2.4% molybdenum and the balance iron. Superior abrasion resistance is achieved by restricting carbon, nickel, chromium, manganese and molybdenum contents to percentages conforming to a limiting mathematical expression of a parabolic effect.

This application is a continuation-in-part of application Ser. No. 403,314, filed Oct. 12, 1964, and now abandoned.

This invention relates to alloys, and especially to white cast irons of a hard, abrasive-resistant type suitable for ball and rod mill liner service, and more particularly characterized as chromium-molybdenum cast irons which may or may not contain nickel.

Ball and rod mills represent processing units important to the mining industry in general, in that such units are necessary for grinding and breaking up ore as mined into finer size incidental to further processing. Such mills are equipped with replaceable liners intended to absorb the severe wear that occurs in the interior of the mill during the course of grinding. The liners are a mosaic of heavy castings bolted or otherwise fastened to the inner surface of the mill, and the alloy of the present invention is particularly suitable as the composition for such liners.

The type of wear experienced by liners of the kind under consideration is characterized as "grinding abrasion" as this term is defined in the publication *Wear*, November-December 1961, vol. 4, No. 6. At times the wear is so severe that as much as one or two pounds of liner metal may be lost by abrasion in the course of milling for every ton of ore ground.

The liners are furnished in various shapes, and may vary in thickness from below two inches to above five inches. Due to the differences in geometry and the severity of operating conditions encountered, including corrosion, a number of problems in metallurgy are presented. Principally, the liner should be of such metallurgical character as to possess both toughness and resistance to abrasion.

Toughness is necessary in order that the liner will withstand chipping tendencies due to the impact from the grinding medium, whether it be ore fragments, balls or rods. Strength and toughness are also required to resist the stress imposed on the liner sections by the weight of the revolving mill load. The need for wear resistance is obvious. Unfortunately the properties of toughness and wear resistance are to a large extent opposite. Thus if an alloy displays superior resistance to wear it may be so brittle as to chip and spall under severe mill action, or the liner sections may fracture after they have worn thin. On the other hand if the alloy is treated or selected to be quite tough and resist both chipping and gross fracture it may wear so rapidly that mill operation is uneconomical.

These tendencies mean that the combination that is best, or in other words, the optimum balance of toughness and abrasion resistance, is a very desirable objective. However, the way to achieve such an objective is not always clear. Hitherto, such optimum balances for mills of different severities have been approximated by selection of alloy types after considerable experience. Austenitic manganese steel and the air-hardening chromium-molybdenum steels are examples of alloys that have been accepted at the tough end of the practical range. Toward the other extreme, where less toughness is needed but where maximum abrasion resistance is economically very desirable, certain cast irons may be acceptable. However, ordinary pearlitic white cast iron seems to lack both toughness and abrasion resistance. Gray cast iron is tough enough for such service as are the ductile irons with spheroidal graphite, but these lack enough abrasion resistance.

There are several alloys on the market which, to a greater or lesser degree, present, at least under given operating conditions, an acceptable balance between toughness and abrasion resistance properties. Toughness may be evaluated in several ways, some of which have been standardized. Thus, the area under the stress-strain curve of a uniaxial tensile test, or the energy absorption from an impact blow (as in the Charpy and Izod techniques), may be used to rank relative toughness. The evaluation of abrasion resistance is more difficult as methods have not been generally standardized and there are recognizably different kinds of abrasive wear. The variables of abrasive hardness, sharpness and toughness; the stress imposed on the metal by the particles of abrasive (which depends on the character of their support); seizing and galling, which are mechanisms that operate under frictional conditions even when no abrasive is present; all contribute to the complexity of wear studies.

Nevertheless, if quantitative evaluation of alloy merit is to be achieved it is necessary to employ a well controlled test that either involves the actual conditions of service or that simulates them satisfactorily. It has been possible to develop a simulated "grinding abrasion" test that has been satisfactorily validated against ball mill service and this test has been important to the evolution of this invention because it permits a scientific prediction of service performance.

Thus, critical consideration of testing for wear resistance is set forth in the above-identified publication, reporting a laboratory test procedure which has been validated by data obtained from actual service testing in a ball mill. The specifications for this test are shown in FIG. 1 hereof, but briefly, a copper lap in the form of a ring track is positioned in a trough that can be filled with a sand and water slurry. The alloy specimen for test is set on the track under a predetermined vertical load, and is submerged in the slurry to the extent that the test abrasive (quartz sand) is crushed between the specimen and the lap or ring in the course of travel of the specimen around the track. The standard for comparison is run at the same time. Weight loss of the specimen provides a measure of wear resistance, reported as wet sand abrasion factor (WSAF) for comparison to the standard which is annealed SAE 1020 steel. A low WSAF signifies a low weight loss, evidencing high abrasion resistance. The reliability of this test has been evaluated satisfactorily many times by replicate runs, which indicate an experimental error range of about plus or minus six percent.

This test does not evaluate the factor of corrosion resistance. In some milling operations the ore, particularly if it contains sulfides, may react with the water also present and form an acid and somewhat corrosive solution. Also some waters may be unusually corrosive. If corro-

sive conditions are present a high level of chromium in the alloy is an asset, since this element is the mainstay of the stainless steels and many corrosion-resistant alloys.

Among the alloys used for ball and rod mill service are the very tough austenitic manganese steels, a variety of hardenable carbon and alloy steels, and several white cast irons. Among the latter are martensitic nickel-chromium and nickel-chromium-molybdenum irons of the so-called "Ni-Hard" alloy type. As stated above, better wear resistance is ordinarily achieved at the sacrifice of toughness, and this is true of the following liner alloys arranged in order of increasing abrasion resistance (decreasing WSAF):

| No.      | Liner Alloy                                  | WSAF ( $\pm 6\%$ ) |
|----------|----------------------------------------------|--------------------|
| (1)..... | Austenitic Manganese Steel.....              | 0.80               |
| (2)..... | Cr-Mo Air-Hardening Steel.....               | 0.70               |
| (3)..... | Martensitic Ni-Cr Cast Iron ("Ni-Hard")..... | 0.55               |

Of the alloys listed above, increasing popularity has favored the martensitic nickel-chromium type (No. 3 above). However, this alloy is not particularly resistant to corrosion, which is a factor to consider in ball mill service, and it is typed as a brittle material. Using a 0.7" square unnotched Charpy type impact specimen for evaluation, values around 7 foot pounds are common.

Some previous experience with a high chromium iron, using a product of tensile strength and elongation as an index of area under the stress strain curve, indicated that it was about twice as tough as the martensitic Ni-Cr iron. Values up to 29 foot pounds have been observed from 0.7 inch square unnotched Charpy specimens.

The structure of martensitic nickel-chromium irons partially accounts for their brittleness, or lack of toughness. Thus, islands or masses of austenite and its transformation products are set in a matrix of brittle iron-carbide which, as the continuous phase, presents little resistance, comparatively speaking, to the propagation of cracks. Hence, the alloy is vulnerable to impact, tension and shear.

High chromium (about 12 to 25% chromium) not only results in corrosion resistance but would reverse the structural pattern of martensitic nickel-chromium cast irons, and yield a generally tougher iron, in that such an alloy is characterized by hard carbides set in a matrix (continuous phase) of austenite or its transformation products which may be martensite, bainite, pearlite or mixtures thereof. A matrix of this character afforded by the high chromium content can be expected to be tougher than that presented by the nickel-chromium martensitic irons. Though favored by toughness and corrosion resistance, the high-chromium irons have hitherto not been sufficiently abrasion resistant to compete economically with the lower alloy irons. This has been especially true of the castings in the heavy sections needed for ball mill liners. It is an important object of this invention to so modify the high chromium irons as to achieve abrasion resistance at least equal to and generally superior to that of the low-chromium or nickel-chromium cast irons, resulting in the favorable balance of properties needed.

Another object of the present invention is to afford an abrasion resistant cast iron alloy in which the resistance to abrasion in thick sections clearly excels the abrasion resistance of alloys of the Ni-Hard type.

Other and further objects of the present invention will be apparent from the following description and claims and are illustrated in the accompanying drawings which, by way of illustration, show preferred embodiments of the present invention and the principles thereof and what is now considered to be the best mode contemplated for applying these principles. Other embodiments of the invention embodying the same or equivalent principles may be used and structural changes may be made as desired by those skilled in the art without departing from the present invention.

In the drawings:

FIG. 1 is a schematic-diagrammatic showing of apparatus and test conditions for a wet sand abrasion factor test; and

FIGS. 2 through 6 are curves showing characteristic features of the alloy of the present invention.

Alloys of the character investigated are sensitive to section thickness, both as cast and after a subsequent heat treatment that may be imposed to develop the metallographic structures that are considered essential to the best abrasion resistance. Heat treatment is almost always considered to be advantageous, and hence is usually included in the foundry specification for alloys of the character involved.

As an example of the sensitivity to section, the wet sand abrasion factors for castings about one inch thick of the martensitic nickel-chromium cast iron type (No. 3 above) may be as low as 0.30, but in the heavier sections (thickness above 2½ inches) despite apparently adequate hardness, the abrasion factors in several commercially produced ball mill liners were found to be as follows:

TABLE 1  
[Martensitic Nickel-Chromium Cast Iron (4.5% Nickel, 1.9% Chromium, 3.2% Carbon)]

| Specimen | Hardness |         | WSAF ( $\pm 6\%$ ) |
|----------|----------|---------|--------------------|
|          | Rc       | BHN     |                    |
| 1.....   | 59.5     | 600     | 0.55               |
| 2.....   | 56.8     | 578     | 0.58               |
| 3.....   | 59.0     | 600     | 0.56               |
| 4.....   | 59.5     | 600     | 0.58               |
| 5.....   | 57-59    | 566-600 | 0.57, 0.56         |
| 6.....   | 57-58    | 555-566 | 0.56, 0.55         |

A similar sensitivity can be seen in Table 5 for alloys of this invention. It may be stated as a caution for those who apply these alloys that hardness, as such, has not been found to be a valid index of resistance to grinding abrasion.

Such a pattern can be universally expected in alloys of the type under consideration. Accordingly, and taking into account experimental error, we consider an abrasion factor (WSAF) at or below 0.60 in a heat treated thick section (5"-6") to represent the criterion of achievement in a high chromium cast iron possessing corrosion resistance, and more toughness, in comparison to a martensitic nickel-chromium alloy of the character identified above.

Table 2 lists 113 experimental compositions determined by us as affording the basis for evaluating the alloy limits of this invention. Each heat was cast in a special mold to simulate the cooling rate of a heavy section thickness, later austenitized at 2000° F. and air cooled at rates characteristic of heavy ball mill liner sections. Abrasion factors (WSAF) and hardness values were then obtained. The WSAF values are for simulated thick or heavy casting (5½" thick). WSAF values for sections of moderate thickness (down to about 1") would be even lower.

TABLE 2.—COMPOSITION, HARDNESS AND ABRASION RESISTANCE OF ALLOYED CAST IRONS FOR BALL MILL LINER SERVICE

| Heat No. | Percent |       |       |      |       |      | After 2,000° F.—<br>2 hours—Air Cool |     |      |
|----------|---------|-------|-------|------|-------|------|--------------------------------------|-----|------|
|          | C       | Mn    | Si    | Ni   | Cr    | Mo   | Rc                                   | BHN | WSAF |
| 1.....   | 3.02    | 0.55  | 0.71  | 0.42 | 19.40 | 1.36 | 62.5                                 | 652 | 0.39 |
| 2.....   | 2.82    | ..... | ..... | 0.63 | 18.50 | 1.76 | 61.0                                 | 652 | 0.40 |
| 3.....   | 2.54    | ..... | ..... | 0.57 | 19.25 | 2.10 | 62.8                                 | 653 | 0.41 |
| 4.....   | 2.53    | ..... | ..... | 0.85 | 19.50 | 1.32 | 61.9                                 | 657 | 0.43 |
| 5.....   | 2.95    | ..... | ..... | 0.57 | 23.50 | 1.28 | 62.2                                 | 652 | 0.43 |
| 6.....   | 2.50    | 0.51  | ..... | 0.88 | 18.90 | 0.81 | 62.0                                 | 652 | 0.43 |
| 7.....   | 2.48    | 0.52  | ..... | 0.82 | 19.25 | 1.75 | 62.5                                 | 653 | 0.44 |
| 8.....   | 2.31    | ..... | ..... | 0.59 | 19.62 | 1.75 | 62.3                                 | 653 | 0.44 |
| 9.....   | 3.03    | ..... | 0.68  | 1.14 | 19.90 | 1.35 | 62.0                                 | 652 | 0.44 |
| 10.....  | 3.10    | 0.51  | ..... | 1.23 | 18.45 | 0.81 | 61.7                                 | 652 | 0.44 |
| 11.....  | 2.82    | 1.43  | 0.75  | 1.23 | 18.25 | 1.77 | 62.1                                 | 627 | 0.44 |
| 12.....  | 2.48    | ..... | ..... | 0.57 | 21.10 | 1.35 | 61.0                                 | 652 | 0.45 |
| 13.....  | 2.97    | 0.53  | ..... | 0.87 | 19.70 | 1.68 | 62.2                                 | 652 | 0.45 |
| 14.....  | 3.31    | ..... | ..... | 0.86 | 19.38 | 1.71 | 62.4                                 | 652 | 0.45 |
| 15.....  | 2.80    | 1.33  | 0.69  | 0.62 | 18.82 | 1.32 | 60.2                                 | 600 | 0.45 |
| 16.....  | 2.75    | 0.51  | ..... | 1.47 | 15.65 | 1.67 | 63.0                                 | 652 | 0.45 |
| 17.....  | 2.83    | 0.53  | 0.69  | 1.43 | 19.30 | 0.78 | 61.5                                 | 627 | 0.45 |

TABLE 2.—Continued

[Heat Treatment: Air Cool from 2,000° F. (1,093° C.)]

| Heat No. | Percent |       |       |       |       |      | After 2,000° F.<br>2 hours—Air Cool |      |      |
|----------|---------|-------|-------|-------|-------|------|-------------------------------------|------|------|
|          | C       | Mn    | Si    | Ni    | Cr    | Mo   | Rc                                  | BHN  | WSAF |
| 18       | 2.75    | 0.49  | ----- | 1.18  | 11.82 | 2.04 | 59.1                                | 578  | 0.45 |
| 19       | 2.84    | 0.52  | 0.63  | 1.14  | 19.35 | 0.75 | 62.1                                | 627  | 0.45 |
| 20       | 2.57    | 0.52  | ----- | 0.84  | 18.08 | 2.38 | 62.6                                | 652  | 0.45 |
| 21       | 2.77    | 1.39  | 0.67  | 0.22  | 19.85 | 1.29 | 61.9                                | 627  | 0.45 |
| 22       | 2.63    | 0.51  | 0.69  | 0.42  | 18.50 | 1.64 | 63.0                                | 652  | 0.46 |
| 23       | 2.46    | 0.51  | ----- | 1.21  | 18.70 | 1.71 | 61.0                                | 639  | 0.46 |
| 24       | 3.18    | ----- | 0.64  | ----- | 18.50 | 1.69 | 59.8                                | 627  | 0.46 |
| 25       | 2.90    | ----- | 0.87  | ----- | 19.30 | 2.04 | 62.3                                | 652  | 0.46 |
| 26       | 2.82    | 1.35  | ----- | 0.90  | 18.90 | 1.49 | 59.1                                | 578  | 0.46 |
| 27       | 3.08    | 0.51  | ----- | 1.36  | 18.78 | 1.36 | 62.1                                | 627  | 0.46 |
| 28       | 2.66    | 1.48  | 0.79  | 0.22  | 18.22 | 1.44 | 62.4                                | 627  | 0.46 |
| 29       | 2.65    | 1.55  | 0.87  | 0.23  | 19.40 | 0.97 | 61.7                                | 627  | 0.46 |
| 30       | 2.72    | ----- | ----- | ----- | 19.20 | 2.11 | 61.8                                | 652  | 0.47 |
| 31       | 2.53    | ----- | 1.07  | ----- | 18.86 | 1.27 | 61.5                                | 639  | 0.47 |
| 32       | 2.85    | 0.50  | 0.71  | 1.43  | 12.65 | 1.69 | 59.2                                | 578  | 0.47 |
| 33       | 3.08    | 0.53  | 0.64  | 1.08  | 19.20 | 1.62 | 61.9                                | 627  | 0.47 |
| 34       | 2.96    | 0.52  | 0.81  | 1.43  | 18.25 | 1.30 | 62.0                                | 652  | 0.47 |
| 35       | 2.76    | 1.65  | 0.70  | 0.74  | 20.09 | 0.95 | 58.2                                | 578  | 0.47 |
| 36       | 2.57    | ----- | 0.57  | ----- | 19.0  | 2.50 | 62.3                                | 652  | 0.48 |
| 37       | 2.99    | ----- | 0.87  | ----- | 19.98 | 1.37 | 62.5                                | 652  | 0.48 |
| 38       | 2.69    | ----- | 0.63  | 1.43  | 20.15 | 1.61 | 62.5                                | 652  | 0.48 |
| 39       | 3.12    | 0.57  | 0.68  | 1.52  | 18.20 | 0.84 | 61.0                                | 600  | 0.48 |
| 40       | 2.70    | 0.52  | ----- | 0.85  | 15.72 | 2.37 | 62.0                                | 627  | 0.48 |
| 41       | 2.86    | 0.53  | ----- | 1.46  | 19.30 | 0.38 | 61.0                                | 600  | 0.48 |
| 42       | 3.23    | 0.52  | ----- | 1.14  | 18.38 | 1.99 | 63.1                                | 652  | 0.48 |
| 43       | 2.37    | ----- | ----- | ----- | 18.08 | 1.67 | 60.9                                | 639  | 0.49 |
| 44       | 2.72    | 0.87  | ----- | 0.56  | 19.54 | 1.32 | 62.2                                | 652  | 0.49 |
| 45       | 2.80    | 0.55  | 0.73  | 0.90  | 18.70 | 0.81 | 63.0                                | 652  | 0.49 |
| 46       | 2.85    | 0.56  | ----- | 0.83  | 25.50 | 0.44 | 59.9                                | 600  | 0.49 |
| 47       | 2.87    | 0.52  | ----- | 1.15  | 15.65 | 1.60 | 59.8                                | 600  | 0.49 |
| 48       | 2.40    | 0.50  | 0.68  | 0.52  | 18.22 | 2.35 | 63.0                                | 652  | 0.49 |
| 49       | 2.65    | 1.04  | ----- | 0.54  | 19.52 | 0.80 | 60.2                                | 600  | 0.49 |
| 50       | 3.03    | 0.48  | ----- | 1.09  | 19.17 | 1.25 | 61.0                                | 627  | 0.49 |
| 51       | 2.97    | 1.28  | 0.91  | 0.14  | 19.50 | 0.90 | 63.0                                | 627  | 0.49 |
| 52       | 2.83    | 1.48  | 1.15  | 0.14  | 17.86 | 1.82 | 63.0                                | 627  | 0.49 |
| 53       | 2.73    | 0.75  | 0.70  | 0.63  | 19.65 | 1.37 | 63.0                                | 652  | 0.49 |
| 54       | 2.60    | ----- | 0.40  | ----- | 19.32 | 1.38 | 61.9                                | 652  | 0.50 |
| 55       | 2.88    | ----- | 0.12  | 19.67 | 2.11  | 62.5 | 652                                 | 0.50 |      |
| 56       | 2.94    | 0.51  | 0.66  | 0.56  | 19.45 | 2.08 | 61.2                                | 627  | 0.50 |
| 57       | 3.14    | 0.53  | ----- | 1.12  | 18.40 | 2.38 | 62.9                                | 652  | 0.50 |
| 58       | 2.52    | 0.52  | 0.95  | 0.81  | 19.42 | 1.30 | 62.8                                | 652  | 0.50 |
| 59       | 2.73    | 0.62  | 0.90  | 1.04  | 18.92 | 1.67 | 62.9                                | 627  | 0.50 |
| 60       | 2.79    | ----- | ----- | ----- | 18.95 | 1.70 | 60.9                                | 639  | 0.51 |
| 61       | 2.65    | ----- | 0.60  | ----- | 22.95 | 1.62 | 62.2                                | 652  | 0.51 |
| 62       | 2.91    | ----- | 0.59  | ----- | 22.40 | 1.66 | 63.0                                | 652  | 0.51 |
| 63       | 2.83    | 0.50  | ----- | 0.42  | 21.90 | 2.05 | 62.5                                | 627  | 0.51 |
| 64       | 3.63    | 0.52  | 0.73  | 1.47  | 18.10 | 1.66 | 60.0                                | 600  | 0.51 |
| 65       | 2.41    | 1.15  | ----- | 0.51  | 19.92 | 0.81 | 59.9                                | 600  | 0.51 |
| 66       | 2.84    | 0.74  | 0.92  | 1.42  | 18.70 | 0.91 | 62.9                                | 627  | 0.51 |
| 67       | 2.56    | 1.43  | 0.78  | 0.55  | 19.83 | 1.81 | 61.6                                | 627  | 0.51 |
| 68       | 2.51    | 0.54  | 0.68  | ----- | 19.95 | 1.69 | 62.8                                | 683  | 0.52 |
| 69       | 2.56    | 0.53  | ----- | 0.62  | 23.55 | 1.42 | 59.5                                | 627  | 0.52 |
| 70       | 2.88    | 0.53  | ----- | 0.90  | 24.95 | 1.61 | 60.5                                | 600  | 0.52 |
| 71       | 2.88    | 1.14  | ----- | 0.82  | 19.64 | 0.81 | 58.3                                | 589  | 0.52 |
| 72       | 2.40    | 0.51  | 0.62  | 1.30  | 20.25 | 0.49 | 61.0                                | 600  | 0.52 |
| 73       | 2.54    | 0.59  | 0.87  | 0.71  | 19.34 | 0.85 | 63.1                                | 627  | 0.52 |
| 74       | 2.77    | ----- | 0.88  | 1.37  | 19.37 | 2.11 | 62.6                                | 627  | 0.53 |
| 75       | 2.83    | 1.37  | 1.02  | 1.24  | 19.30 | 1.47 | 59.6                                | 589  | 0.53 |
| 76       | 2.69    | 0.46  | 0.95  | 0.82  | 18.28 | 2.03 | 62.9                                | 652  | 0.53 |
| 77       | 2.63    | 1.51  | 0.81  | 0.67  | 19.42 | 1.35 | 58.4                                | 578  | 0.53 |
| 78       | 2.64    | 0.47  | ----- | 1.38  | 18.57 | 1.25 | 61.9                                | 630  | 0.54 |
| 79       | 2.57    | 0.68  | 0.77  | 0.87  | 19.75 | 1.32 | 62.5                                | 652  | 0.54 |
| 80       | 2.68    | ----- | 0.58  | 20.45 | 1.32  | 62.5 | 652                                 | 0.55 |      |
| 81       | 3.00    | 0.53  | ----- | 0.39  | 12.50 | 2.03 | 56.0                                | 532  | 0.55 |
| 82       | 2.46    | 1.24  | 0.90  | 0.97  | 19.55 | 0.53 | 62.0                                | 613  | 0.55 |
| 83       | 2.62    | 1.38  | 0.96  | 0.96  | 19.25 | 0.92 | 61.0                                | 600  | 0.55 |
| 84       | 2.77    | 0.52  | 0.73  | 0.85  | 15.65 | 1.61 | 59.6                                | 600  | 0.56 |
| 85       | 2.86    | 0.53  | ----- | 0.90  | 24.95 | 1.61 | 60.5                                | 600  | 0.56 |
| 86       | 2.12    | 0.65  | 0.77  | 0.69  | 20.10 | 0.86 | 61.9                                | 627  | 0.56 |
| 87       | 3.03    | 0.53  | ----- | 0.40  | 22.80 | 0.81 | 62.0                                | 600  | 0.57 |
| 88       | 2.88    | 0.49  | 0.74  | 0.37  | 12.20 | 1.20 | 57.0                                | 555  | 0.57 |
| 89       | 2.72    | ----- | 0.42  | 19.95 | 0.87  | 61.6 | 652                                 | 0.58 |      |
| 90       | 2.38    | 0.52  | 0.75  | 0.40  | 19.20 | 1.49 | 63.0                                | 683  | 0.58 |
| 91       | 3.17    | 0.55  | 0.71  | 0.91  | 18.95 | 0.82 | 62.0                                | 652  | 0.58 |
| 92       | 3.17    | 0.61  | 0.55  | 0.79  | 17.80 | 1.08 | 60.7                                | 600  | 0.58 |
| 93       | 2.38    | 0.52  | ----- | 1.10  | 19.09 | 1.30 | 62.5                                | 652  | 0.58 |
| 94       | 2.33    | 0.51  | 0.68  | 0.76  | 18.85 | 1.98 | 62.3                                | 652  | 0.58 |
| 95       | 2.74    | 0.52  | ----- | 0.85  | 16.15 | 1.21 | 60.4                                | 600  | 0.60 |
| 96       | 3.32    | ----- | 0.56  | 19.98 | 1.33  | 61.4 | 613                                 | 0.62 |      |
| 97       | 3.10    | 0.52  | ----- | 0.56  | 19.80 | 1.32 | 61.0                                | 600  | 0.62 |
| 98       | 3.01    | 0.55  | 0.62  | 0.62  | 20.15 | 0.78 | 61.1                                | 627  | 0.63 |
| 99       | 2.81    | 0.53  | 1.06  | 0.62  | 19.02 | 1.27 | 61.0                                | 600  | 0.64 |
| 100      | 2.47    | ----- | 0.66  | 16.93 | 1.35  | 57.4 | 600                                 | 0.67 |      |
| 101      | 2.47    | ----- | 1.05  | 0.56  | 12.80 | 1.32 | 56.2                                | 555  | 0.68 |
| 102      | 2.98    | ----- | ----- | ----- | 19.73 | 1.67 | 60.7                                | 627  | 0.70 |
| 103      | 3.38    | 0.51  | ----- | 0.59  | 19.34 | 1.74 | 60.0                                | 627  | 0.70 |
| 104      | 2.95    | ----- | 0.71  | 0.53  | 16.40 | 1.65 | 55.2                                | 532  | 0.70 |
| 105      | 2.99    | ----- | 0.65  | 0.54  | 17.60 | 1.35 | 55.2                                | 555  | 0.71 |
| 106      | 2.78    | ----- | ----- | ----- | 20.00 | 1.61 | 60.5                                | 600  | 0.72 |
| 107      | 2.54    | ----- | 0.57  | 19.76 | 0.42  | 45.3 | 444                                 | 0.76 |      |
| 108      | 2.96    | 0.52  | 0.72  | ----- | 18.75 | 1.71 | 55.2                                | 555  | 0.77 |
| 109      | 2.56    | ----- | ----- | ----- | 19.73 | 1.30 | 51.0                                | 495  | 0.78 |
| 110      | 3.21    | ----- | 0.52  | 19.98 | 0.79  | 48.2 | 460                                 | 0.79 |      |
| 111      | 2.70    | ----- | 0.39  | 20.52 | 0.44  | 53.5 | 532                                 | 0.82 |      |
| 112      | 2.79    | ----- | ----- | 18.20 | 0.83  | 44.5 | 437                                 | 0.84 |      |

The order of experimental alloys in Table 2 is established on the basis of their wet sand abrasion factors (WSAF) and any alloy having a WSAF above 0.60 is arbitrarily rated as unacceptable. (This is not necessarily a practical limitation because some alloys widely

used for ball mill liners have WSAF values above 0.60.) The WSAF value of 0.60 is about the upper edge of the band established by the plus or minus 6% experimental error of the abrasion test when applied to the values in Table 1 for nickel-chromium irons.

It is apparent that there is no simple correlation among the alloy elements carbon, chromium, molybdenum and nickel. This is more apparent from FIGS. 2 and 3, which show that with increasing additions of nickel and molybdenum, superior wear resistance is gradually achieved up to a certain value, but that with further additions beyond this value a reversal of effect is encountered leading toward an unacceptable abrasion factor.

Similar curves are found for the effect of carbon and chromium, indicating that an over-all parabolic effect prevails, such that there is no easily predictable parameter for selection of the allow ingredients. However, based on previous experience and judicious balancing of factors, we determined the composition ranges for WSAF of 0.60 or less to be (balance, substantially iron):

C, percent ----- 2.1-3.4  
Ni, percent ----- 0-1.6  
Cr, percent ----- 12.5-25.6  
Mo, percent ----- 0.38-2.90

Manganese can be present up to at least about 2% and silicon up to about 1.2%.

Examination of the last seventeen heats in Table 2, however, shows that these heats do not subscribe to the basic requirement of an abrasion factor of 0.60 or less. In fact, from a study of eighty-six selected heats it was postulated that there were no less than fourteen interactions among the four significant variables (carbon, chromium, nickel and molybdenum) to be weighted and taken into account in any realistic effort to determine the parameters of an acceptable alloy (using a WSAF value of 0.60 or less as the dependent variable) under the present invention.

Based on these interactions and the observed parabolic relation, it is found that the composition range set forth above is acceptable so long as the percentages of the four variables in the following formula produce a calculated value for WSAF that does not exceed the desired value of 0.60:

$$\begin{aligned}
 WSAF = & 4.33723 - 0.91600 \times C\% \\
 & - 0.55522 \times Ni\% \\
 & - 0.14862 \times Cr\% \\
 & - 1.06313 \times Mo\% \\
 & + 0.19926 \times (C\% \times C\%) \\
 & - 0.25780 \times (C\% \times Ni\%) \\
 & + 0.00397 \times (C\% \times Cr\%) \\
 & - 0.02825 \times (C\% \times Mo\%) \\
 & + 0.19056 \times (Ni\% \times Ni\%) \\
 & + 0.02360 \times (Ni\% \times Cr\%) \\
 & + 0.26964 \times (Ni\% \times Mo\%) \\
 & + 0.00168 \times (Cr\% \times Cr\%) \\
 & + 0.03104 \times (Cr\% \times Mo\%) \\
 & + 0.08838 \times (Mo\% \times Mo\%)
 \end{aligned}$$

Thus, it is found that when a graph of calculated versus observed WSAF is made, all of the WSAF values for the eighty-six selected heats used to determine the above formula fall within a plus or minus 22% scatter band of observed WSAF, which band is merely a profile of the

extent of error in such factors as chemical analysis, testing for WSAF ( $\pm 6\%$ ), foundry limitations, and metallurgical processing, thereby confirming Formula 1 within expected experimental error.

Applicability of Formula 1 to foundry specifications can be visualized from the parabolas of FIGS. 4 and 5 (calculated) which, incidentally, are validated by the parabolas of FIGS. 2 and 3, confirming Formula 1. For FIG. 4, the assumed cast iron composition included 2.8% carbon, 19.00% chromium and 1.00% molybdenum as a base. WSAF values were then calculated by Formula 1 and plotted for the nickel amounts shown. FIG. 4, then, indicates that for such a basic cast iron, superior wear resistance is achieved with 1.45% nickel. Below 0.6% or above 2.3% nickel, the chances are poor of obtaining an abrasion factor below 0.60.

Similarly, according to FIG. 5, acceptable performance can be expected from an alloy analyzing about 2.8% carbon, 26.0% chromium, 0.40% molybdenum, 0.3-2.6% nickel, balance substantially iron.

The heats listed in Table 2 were experimental heats which served as a basis for determination of the above formula that qualifies the working foundry specification. Actual mill liners were cast from the following heat:

TABLE 3

| Heat 507: | Percent |
|-----------|---------|
| C         | 3.15    |
| Mn        | 0.76    |
| Si        | 0.65    |
| Cr        | 19.70   |
| Mo        | 1.25    |
| Ni        | 0.71    |
| P         | 0.014   |
| S         | 0.012   |

and resulted in the following observed data (after 2000° F. for six hours, air cool):

TABLE 4

| Specimen Location       | Hardness |     | WSAF<br>(Observed) |
|-------------------------|----------|-----|--------------------|
|                         | Rc       | BHN |                    |
| Surface of 2½" section  | 62.9     | 652 | 0.35               |
| Interior of 2½" section | 62.5     | 626 | 0.38               |
| Surface of 5¼" section  | 63.1     | 667 | 0.33               |
| Interior of 5¼" section | 62.9     | 627 | 0.49               |

The following are data pertaining to full scale production heats for ball mill liners:

TABLE 5

| Heat   | Properties After Heat Treatment (2,000° F.—Air Cool) |      |      |       |       |      |               |      |      |          |      |      |               |      |      |          |      |      |
|--------|------------------------------------------------------|------|------|-------|-------|------|---------------|------|------|----------|------|------|---------------|------|------|----------|------|------|
|        | Percent                                              |      |      |       |       |      | Light Section |      |      |          |      |      | Heavy Section |      |      |          |      |      |
|        | C                                                    | Mn   | Si   | Ni    | Cr    | Mo   | Surface       |      |      | Interior |      |      | Surface       |      |      | Interior |      |      |
|        |                                                      |      |      |       |       |      | Rc            | BHN  | WSAF | Rc       | BHN  | WSAF | Rc            | BHN  | WSAF | Rc       | BHN  | WSAF |
| 184    | 2.47                                                 | 0.75 | 0.62 | 0.73  | 19.82 | 0.73 | 63            | 652  | 0.45 | 63       | 652  | 0.44 | 63            | 652  | 0.58 | 62       | 627  | 0.60 |
| 188    | 2.95                                                 | 0.73 | 0.73 | 0.77  | 19.09 | 1.14 | 60            | 600  | 0.36 | 58       | 555  | 0.39 | 63            | 652  | 0.36 | 61       | 627  | 0.42 |
| AJ 552 | 2.83                                                 | 0.71 | 1.24 | 19.54 | 1.27  | 65   | 633           | 0.35 | 64   | 652      | 0.43 | 64   | 633           | 0.37 | 64   | 652      | 0.53 |      |
| 128    | 2.89                                                 | 0.70 | 0.47 | 0.54  | 18.12 | 1.38 |               |      |      | 63       | 652  | 0.43 | 64            | 652  | 0.51 |          |      |      |

The effect of section thickness and close correspondence of calculated versus observed WSAF values can be seen from the following data, wherein the light sections were of 2½" thickness and the heavy sections of 5½" thickness:

TABLE 6

| Heat   | Calculated WSAF<br>(Heavy section) | Actual WSAF   |          |               |          |
|--------|------------------------------------|---------------|----------|---------------|----------|
|        |                                    | Light Section |          | Heavy Section |          |
|        |                                    | Surface       | Interior | Surface       | Interior |
| 507    | 0.56                               | 0.35          | 0.38     | 0.33          | 0.49     |
| 188    | 0.52                               | 0.36          | 0.39     | 0.36          | 0.42     |
| AJ 552 | 0.46                               | 0.35          | 0.43     | 0.37          | 0.53     |

Manganese and silicon may be employed in the nominal amounts of 0.5% and 0.6% respectively, but may be

varied from about 0.4-2.0% and 0.2-1.2%, respectively. Carbon, chromium, molybdenum and nickel are calculated by means of the parabola Formula No. 1 above; but Formula No. 2, hereinafter, is also valid.

Since the apex of the parabola represents the optimum alloy when three elements are held constant and the other is varied, it is apparent that a great variety of alloys can be calculated with the broad composition limits given and that many different optimum values could be selected. In general, the optimum is selected by inspection after plotting the calculated points from the base composition selected to bracket the apex of the parabola. However, a foundry ordinarily wishes a less mathematically involved specification. At the same time a reasonable melting range is needed to allow for the production variables that cannot ordinarily be avoided. Obviously, the wide limits of the broad range of this invention cannot be used for this purpose as many of the resultant alloys, as melted in the foundry, would fall outside the restrictions imposed by the formula.

To aid the foundry that is to produce the highly abrasion-resistant alloys that are intended, either an aim point on a production range can be specified, and a number of these aim points are specified as claims herein. Where one element is shown as a variable it can be aimed at the center of the range given if the optimum product is desired. On the other hand, if a more economical specification is desired the variable element can be aimed within the low side of the range given, but not outside the extreme limits.

If a simple six-element production range is desired, the following production specification is provided as an example, one judiciously selected to provide reasonable assurance that the alloy of the present invention will be realized without recourse to the rather tedious mathematical calculations of the formula:

|             |           |
|-------------|-----------|
| C, percent  | 2.5-3.5   |
| Mn, percent | 0.4-1.7   |
| Si, percent | 0.2-1.2   |
| Cr, percent | 17.0-21.0 |
| Ni, percent | 0.3-0.9   |
| Mo, percent | 1.0-1.7   |

In practice, the foundry would aim at the approximate midpoints of these ranges. Because of normal variations in charge make-up and melting conditions the end result of each melt will inevitably vary somewhat from this aim.

If all of the elements should fortuitously fall on the low side of the ranges above, the expected abrasion factor would fall well up on the parabola away from the apex and the expected abrasion factor would be above 0.60. However, it is very unlikely that all elements would vary in this way. Their variation is expected to be random and if one is low, then another may well be expected to be high. Also, the extreme variations are much less likely than small departures from the aim point.

Note that under the production specification set forth immediately above, if molybdenum should fall so low as 1.0%, it can be deduced from FIG. 4 that with the aim point of 0.6% nickel a factor of 0.60 or better is still possible. On the other hand, if nickel should fall as low as 0.3% or 0.4%, from FIG. 3 it may be deduced that the

aim point of 1.35% molybdenum would still produce an expected abrasion factor of 0.51.

This practical specification takes into account the fact that nickel and molybdenum losses in melting are usually lower than those of chromium and manganese, and thus these elements are less likely to vary much from the aim point. However, if one or more elements are outside the ranges given, the melt may be arbitrarily rejected as probably inferior unless the producer wishes to apply the formula to determine acceptability. If two of the elements (in the group of carbon, chromium, molybdenum and nickel) are below the limits shown it is not considered likely that compensation by means of the other two will be great enough to avoid inferior abrasion resistance.

The elements manganese and silicon have a somewhat different status. The ranges shown have been found by experiment to produce acceptable results and they are given here because nearly all foundries prefer to specify and monitor these. Practically, they can be held to closer limits than the ones shown; and with good melting practice and the suggested aim points of 0.5% manganese and 0.6% silicon there is little likelihood that final results will reach the extremes of the foundry specification.

It should be apparent that many other suitable foundry specifications can be developed with the aid of the formula and the parabolic plots that it makes possible. Narrow ranges are desirable to provide the maximum likelihood of best abrasion resistance. Where a foundry knows its own melting variations, it would be advisable to use these as the basis of limits in a practical foundry specification that is centered on the apex of the parabola, where each element in turn is plotted as the variable and the other three are fixed.

The practical foundry specification should also call for heat treatment at 2000° F. followed by air cooling. This was used as a convenient method of microstructural control to achieve the balance discovered to be effective by abrasion testing and implied by the formula. However, this does not preclude the use of other temperatures for heat treatment or the use of the alloy as-cast. If the cooling and constituent balance are right for the section thickness involved, a desirable high level of resistance to high stress grinding abrasion is attainable, provided the alloy is made as described by the formula. If a thermal history other than the one described here is in prospect its merits can be evaluated by the abrasion test as embodied in FIG. 1.

It should be recognized that there are other types of abrasion. The high-chromium irons generally have been found to be resistant to erosion or low-stress scratching abrasion in both service and laboratory tests. They have also performed well in a test against the abrasion of an Alundum grinding wheel. The laboratory erosion tests on several alloys made according to the formula described here indicated that they had from 12 to 28 times the resistance to such wear as the standard of SAE 1020 steel. One alloy was 15 times as resistant in the as-cast state.

While the alloy featured here was developed primarily for ball and rod mill grinding service the other tests that have been made indicate that it has wide potential usefulness as a general purpose abrasion resistant alloy. It is not intended that its use will be restricted to mills. Many service environments include several types of abrasion (as well as various levels of impact or other stresses) and the alloy described here can be expected to provide superior resistance to the high-stress abrasion component as well as very good resistance to the other aspects of abrasion.

In the derivation of Formula 1, the computer was not programmed to consider the effect of manganese, and Formula 1 is most valid for a manganese content of about 0.5%. However, eighty-seven additional heats were made in which manganese was deliberately varied, these

70  
75

heats falling within the following limits, balance substantially all iron with silicon at a nominal 0.6% level:

|             |           |
|-------------|-----------|
| C, percent  | 2.5-3.2   |
| Mn, percent | 0.4-2.1   |
| Ni, percent | 0.1-1.9   |
| Cr, percent | 15.0-23.0 |
| Mo, percent | 0.4-2.4   |

As to these heats, the average WSAF value was about 0.5366. It was found that manganese conforms to and presents substantially the parabolic effect, and in fact studies reveal that a formula which takes manganese into account as a variable subscribes to the following formula where the value for WSAF does not exceed the desired value of 0.60:

### Formula 2

$$\begin{aligned}
 WSAF = & 4.36628 - 1.28656 \times C\% \\
 & - 0.80306 \times Mn\% \\
 & - 1.11022 \times Ni\% \\
 & - 0.15963 \times Cr\% \\
 & - 0.94015 \times Mo\% \\
 & - 0.19451 \times (C\% \times Mn\%) \\
 & - 0.22763 \times (C\% \times Ni\%) \\
 & - 0.01185 \times (C\% \times Cr\%) \\
 & + 0.02301 \times (C\% \times Mo\%) \\
 & + 0.31381 \times (Mn\% \times Ni\%) \\
 & + 0.04159 \times (Mn\% \times Cr\%) \\
 & + 0.12577 \times (Mn\% \times Mo\%) \\
 & + 0.03510 \times (Ni\% \times Cr\%) \\
 & + 0.27389 \times (Ni\% \times Mo\%) \\
 & + 0.01329 \times (Cr\% \times Mo\%) \\
 & + 0.30712 \times (C\% \times C\%) \\
 & + 0.06573 \times (Mn\% \times Mn\%) \\
 & + 0.25418 \times (Ni\% \times Ni\%) \\
 & + 0.00308 \times (Cr\% \times Cr\%) \\
 & + 0.08836 \times (Mo\% \times Mo\%)
 \end{aligned}$$

Formula 2 is of particular value in determining substitutions of manganese (cheaper) for molybdenum (more expensive).

Hence, while we have illustrated and described preferred embodiments of our invention, it is to be understood that these are capable of variation and modification.

We claim:

1. An abrasion resistant cast iron consisting essentially of about 2.5 to 3.4% carbon, 0.15 to 1.6% nickel, 12.5 to 25.6% chromium and 0.38 to 2.90% molybdenum, balance substantially all iron, and in which the actual percentages of carbon, chromium, nickel and molybdenum do not produce a calculated value of more than 0.60 under the formula:

$$\begin{aligned}
 WSAF = & 4.33723 - 0.91600 \times C\% \\
 & - 0.55522 \times Ni\% \\
 & - 0.14862 \times Cr\% \\
 & - 1.06313 \times Mo\% \\
 & + 0.19926 \times (C\% \times C\%) \\
 & - 0.25780 \times (C\% \times Ni\%) \\
 & + 0.00397 \times (C\% \times Cr\%) \\
 & - 0.02825 \times (C\% \times Mo\%) \\
 & + 0.19056 \times (Ni\% \times Ni\%) \\
 & + 0.02360 \times (Ni\% \times Cr\%) \\
 & + 0.26964 \times (Ni\% \times Mo\%) \\
 & + 0.00168 \times (Cr\% \times Cr\%) \\
 & + 0.03104 \times (Cr\% \times Mo\%) \\
 & + 0.08838 \times (Mo\% \times Mo\%)
 \end{aligned}$$

2. An abrasion resistant cast iron alloy consisting essentially of about 2.8% carbon, 19% chromium, 1.3% molybdenum, 0.5% manganese, 0.6% silicon and 0.15 to 1.16% nickel, balance substantially all iron.

3. An abrasion resistant cast iron alloy consisting essentially of about 2.6% carbon, 19% chromium, 0.4% nickel, 0.5% manganese, 0.6% silicon, and 0.7-2.9% molybdenum, balance substantially all iron.

4. An abrasion resistant cast iron alloy consisting essentially of about 2.8% carbon, 19% chromium, 1.0% molybdenum, 0.5% manganese, 0.6% silicon and 0.5-2.4% nickel, balance substantially all iron.

5. An abrasion resistant iron alloy consisting essentially of about 2.8% carbon, 26.0% chromium, 0.4% molybdenum, 0.5% manganese, 0.6% silicon, and 0.3 to 2.6% nickel, balance substantially all iron.

6. An abrasion resistant cast iron alloy consisting essentially of about 2.8% carbon, 26.0% chromium, 0.4% molybdenum and 1.5% nickel, balance substantially all iron.

7. An abrasion resistant cast iron alloy consisting essentially of about 2.8% carbon, 19% chromium, 0.75% nickel, and 2% molybdenum, balance substantially all iron.

8. An abrasion resistant cast iron alloy consisting essentially of about 2.8% carbon, 19% chromium, 1.0% nickel, and 1.6% molybdenum, balance substantially all iron.

9. An abrasion resistant cast iron alloy consisting essentially of about 3.1% carbon, 0.5% manganese, 0.6% silicon, 19% chromium, 0.5% nickel and 1.2% molybdenum, balance substantially all iron.

10. An abrasion resistant cast iron alloy according to claim 1 in the form of a grinding mill liner.

11. An abrasion resistant cast iron consisting essentially of about 2.5 to 3.2% carbon, 0.4 to 2.1% manganese, 0.1 to 1.9% nickel, 15 to 23% chromium, and 0.4 to 2.4% molybdenum, balance substantially all iron, and in which the actual percentages of carbon, manganese, chromium, nickel and molybdenum do not produce

a calculated value of more than 0.60 under the formula:

$$\begin{aligned}
 WSAF = & 5.36628 - 1.28656 \times C\% \\
 & - 0.80306 \times Mn\% \\
 & - 1.11022 \times Ni\% \\
 & - 0.15963 \times Cr\% \\
 & - 0.94016 \times Mo\% \\
 & - 0.19451 \times (C\% \times Mn\%) \\
 & - 0.22763 \times (C\% \times Ni\%) \\
 & - 0.01185 \times (C\% \times Cr\%) \\
 & + 0.02301 \times (C\% \times Mo\%) \\
 & + 0.31381 \times (Mn\% \times Ni\%) \\
 & + 0.04159 \times (Mn\% \times Cr\%) \\
 & + 0.12577 \times (Mn\% \times Mo\%) \\
 & + 0.03510 \times (Ni\% \times Cr\%) \\
 & + 0.27389 \times (Ni\% \times Mo\%) \\
 & + 0.01329 \times (Cr\% \times Mo\%) \\
 & + 0.30712 \times (C\% \times C\%) \\
 & + 0.06573 \times (Mn\% \times Mn\%) \\
 & + 0.25418 \times (Ni\% \times Ni\%) \\
 & + 0.00308 \times (Cr\% \times Cr\%) \\
 & + 0.08836 \times (Mo\% \times Mo\%)
 \end{aligned}$$

12. An abrasion resistant cast iron alloy according to claim 11 in the form of a grinding mill liner.

#### References Cited

##### UNITED STATES PATENTS

|           |         |         |       |          |
|-----------|---------|---------|-------|----------|
| 2,253,873 | 8/1941  | Trantin | ----- | 75—126 X |
| 2,355,726 | 8/1944  | Hardes  | ----- | 75—126   |
| 2,773,761 | 12/1956 | Fuqua   | ----- | 75—126   |

##### FOREIGN PATENTS

|         |        |          |
|---------|--------|----------|
| 162,179 | 9/1964 | U.S.S.R. |
|---------|--------|----------|

L. DEWAYNE RUTLEDGE, Primary Examiner.

P. WEINSTEIN, Assistant Examiner.

UNITED STATES PATENT OFFICE  
CERTIFICATE OF CORRECTION

Patent No. 3,410,682

November 12, 196

Howard S. Avery et al.

It is certified that error appears in the above identified patent and that said Letters Patent are hereby corrected as shown below:

Column 10, line 20, "WSAF=4.36628-1.28656xC%" should read -- WSAF=5.36628-1.28656 X C% --. Column 12, line 6, "-0.94016 X Mo%" should read -- -0.94015 X Mo% --.

Signed and sealed this 17th day of March 1970.

(SEAL)

Attest:

Edward M. Fletcher, Jr.

Attesting Officer

WILLIAM E. SCHUYLER, JR.

Commissioner of Patents